

UNITED STATES PATENT OFFICE.

THOMAS H. DENNEY, OF CAPE CHARLES, VIRGINIA, ASSIGNOR TO LEONARD J. WHITEHEAD AND JAMES B. JONES, OF CAPE CHARLES, VIRGINIA, AND JOSEPHUS F. BUSSELLS, OF IRVINGTON, VIRGINIA.

ANTIFOULING PAINT.

SPECIFICATION forming part of Letters Patent No. 715,763, dated December 16, 1902.

Application filed November 27, 1901. Serial No. 83,908. (No specimens.)

*To all whom it may concern:*

Be it known that I, THOMAS H. DENNEY, a citizen of the United States, residing at Cape Charles, in the county of Northampton and State of Virginia, have invented certain new and useful Improvements in Antifouling Paints; and I do declare the following to be a full, clear, and exact description of the invention, such as will enable others skilled in the art to which it appertains to make and use the same.

My invention relates to improvements in antifouling paints in which mercury is employed as an active element for the destruction of marine growths.

The object of the invention is to produce an antifouling compound that can be applied over metal or other surfaces without deleterious action thereon, and to accomplish this end by employing mercury as the antifouling agent by so combining it with other ingredients as to require but a comparatively small quantity thereof, due primarily to the absence of neutralizing ingredients and to effective distribution and suspension of the mercury in the compound, as well as by reason of its protection therein against too-rapid action and consequent consumption, thereby rendering the compound lasting and the use of mercury therein commercially profitable.

The use of mercury in antifouling compounds has been usually limited to that of an auxiliary agent on account of its expensiveness and the difficulty in effectually combining it, the combination being usually effected by employing mercury in other than its native form, with the result of a loss in its active properties. Moreover, it has been a common source of error to combine the mercury with ingredients which have a neutralizing effect upon it, such as iron and other metal. With these considerations in view the present invention aims to make a practical advance in this art and has as a chief concern the production of a coating compound for the bottoms of iron or steel vessels which will be suitable for application over the usual coating of red lead and act as a seal therefor against the dissolving and softening

action of the sea-water while performing its antifouling function.

The invention consists in the formation of a paste of mercury, tallow, ocher, linseed-oil, and drier to be handled commercially and used with the addition of red lead, the same being compounded substantially as herein-after set forth in order that when applied it will remain in a semidry state hard enough to resist the washing action of the sea, yet be subject to such gradual dissolution as to keep it always active.

In compounding the above-named ingredients I employ mercury in its native state in order to render the galvanic action freer, and with the requisite quantity thereof is mixed heated tallow, the melted tallow allowing the mercury to be thoroughly mixed therewith, and when cooled during the mixing to hold the mercury in suspension, as well as forming a preservative body that will prevent the compound from drying hard and leaving the mercury either exposed to too-rapid consumption or so incased by the formation of an outer skin as to be wholly or partially inactive. The mixing of the mercury and tallow is preferably accomplished in a bur-mill. Ocher is employed as a base for the paste, and the requisite quantity thereof is mixed with linseed-oil and drier, after which these three ingredients so incorporated are added to the mercury and tallow and the entire mass mixed until a thorough incorporation of all the ingredients takes place. By this manner of mixing the ingredients not only is the incorporation thereof thorough, but the whole mass is rendered so as to make separation of the ingredients impossible. The result is a thick paste which can be commercially handled without danger of deterioration and which requires the subsequent addition of dry red lead for the twofold purpose of causing the paste to harden sufficiently when applied and to cause it to adhere especially over a coating of red lead by reason of the affiliation of the lead in the paste with that of the coating.

In making this compound I found it effective to combine the ingredients in the following proportions to make about twenty-five gallons

of the compound: mercury, seventeen pounds; tallow, twenty-five pounds; ocher, one hundred and twenty-eight pounds; linseed-oil, eight gallons; Japan drier, two gallons; red lead, twenty-five pounds. Though the compound formed by these ingredients in the quantities substantially as here given is in the form of a thick paste, it is adapted to be applied by a brush and is effectively spread thereby so as to form an even coating of the required thickness. As before stated, the consistency of the paint is important in preserving a thorough incorporation of the several ingredients not only when the paste is applied, but when the

same is being commercially handled, while the dry red lead is necessary to bring it into a semidry condition, but cannot be added except as the compound is being used.

What I claim is—

An antifouling paint consisting of mercury, tallow, ocher, linseed-oil, drier and red lead, combined substantially as herein described.

In testimony whereof I affix my signature in presence of two witnesses.

THOMAS H. DENNEY.

Witnesses:

THOMAS J. WESCOTT,  
CLARENCE G. SMITHERS.